

# UNITED STATES PATENT OFFICE.

ALVAH W. CLEMENT, OF CLEVELAND, OHIO, ASSIGNOR TO THE CLEVELAND BRASS MANUFACTURING COMPANY, OF CLEVELAND, OHIO, A CORPORATION OF OHIO.

## ACID-RESISTING ALLOY.

1,375,672.

Specification of Letters Patent. Patented Apr. 26, 1921.

No Drawing.

Application filed July 26, 1917. Serial No. 182,911.

*To all whom it may concern:*

Be it known that I, ALVAH W. CLEMENT, a citizen of the United States, residing at Cleveland, in the county of Cuyahoga and 5 State of Ohio, have invented a certain new and useful Improvement in Acid-Resisting Alloys, (B,) of which the following is a full, clear, and exact description.

This invention relates to metal alloys, and 10 seeks to provide an alloy of metals, which alloy shall be highly resistant to acid, particularly nitric acid, even though the acid be in a hot dilute condition.

Such an alloy may be utilized to provide 15 stills, nitrators, containers, pumps, pipes and cocks, and other articles by which the acid may be handled in a manner similar to pipe lines for conducting water or other fluids.

20 The alloy herein proposed, consists substantially of chromium, iron and carbon in the proportion of substantially 60 per cent. of chromium, substantially 2 to 5 per cent. of carbon, substantially 2 to 4 per cent. of silicon, and the remainder of iron.

The carbon in this alloy exists mainly in its uncombined or graphitic form.

In the preparation and fusing of the com-

ponent parts of the alloy, silicon may be used in order to render the alloy more fluid 30 than it otherwise would be, thus making it easier to handle. The silicon also has the property of causing the carbon which may be contained in the fused chromium and iron to assume the form of graphitic carbon when the alloy is finally cooled. The amount of silicon thus used will vary up 35 to substantially 4 per cent.

The alloy must be practically free of manganese or other elements which tend to 40 counteract the action of silicon.

The alloy thus formed will be highly resistant to nitric acid, hot or cold, concentrated or dilute.

Having thus described my invention, what 45 I claim is:

An acid resisting alloy consisting of substantially 60 per cent. chromium, substantially 2 to 4 per cent. silicon, substantially 2 to 5 per cent. carbon existing in the alloy 50 as graphitic carbon, and the remainder of iron.

In testimony whereof, I hereunto affix my signature.

ALVAH W. CLEMENT.